

(No Model.)

H. P. FOLSOM.

RANGE BOILER.

No. 307,852.

Patented Nov. 11, 1884.



Witnesses:  
H. F. Parker.  
Joseph Martin -

Inventor:  
Henry P. Folsom  
by  
C. W. Phelps Betts  
Attorney.

# UNITED STATES PATENT OFFICE.

HENRY P. FOLSON, OF BROOKLYN, NEW YORK.

## RANGE-BOILER.

SPECIFICATION forming part of Letters Patent No. 307,852, dated November 11, 1884.

Application filed December 19, 1883. (No model.)

*To all whom it may concern:*

Be it known that I, HENRY P. FOLSON, of the city of Brooklyn, county of Kings, State of New York, have invented certain new and 5 useful Improvements in Range-Boilers and other similar Vessels to be Used under Pressure, of which the following is a full, clear, and exact description, reference being had to the accompanying drawing, forming part of the 10 annexed specification.

My invention consists of a closed metallic vessel, suitable for containing liquids under pressure, which is continuously enameled or glazed throughout with a fused surface-glaze. 15 In the drawing is shown a section of my improved range-boiler, in which drawing A represents the outer cylinder, B B' the two heads, and C C C the continuous inside enameling or fused glaze, and D D a similar outside 20 enameling.

Prior to my invention range-boilers have been made in a variety of ways. Ordinarily such boilers have been made of iron galvanized; but these boilers last but a comparatively 25 short time, owing to the imperfection of the galvanizing process, as many parts of the boilers and shells are imperfectly coated and the zinc scales off and presents a surface to permit rust. The galvanizing has no effect in 30 strengthening the boilers. Boilers have also been made of iron lined with copper. Boilers of this kind are very expensive, owing to the necessity of forming a complete inner vessel of copper, and owing to the difficulty of making 35 such inner vessel perfectly tight without very great expense. Such boilers are also liable to rapid deterioration from rust affecting the iron. Boilers have also been made entirely of copper; but these, owing to the character of the 40 material, are quite liable to collapse, and any boiler in which the inner surface is copper is apt to injure the water contained in it by the precipitation of oxide of copper. Boilers have also been made with a coating of enamel on 45 the inside, which partially remedies the difficulties alluded to, as shown in Letters Patent to Charles H. Buck, March 17, 1874, No. 148,593; but such boilers are still open to objections. The Buck boiler is made with the 50 bottom and top heads of cast-iron, while the cylinder only is made of sheet-iron. This is

quite expensive, and at the same time does not secure a perfect homogeneity of material, and prevents the seams from being made as tight as in my method. Buck also speaks of enameling his boiler; but the enamel which he uses, in common with all enameled similar vessels prior to my invention, is ordinary white enamel. This enamel is so composed that it does not secure a perfect adhesion between the 55 enamel and the surface of the boiler, so that the enamel is liable to crack off, especially at the joints where it is most needed.

Neither does Buck, or any inventor prior to the date of my invention, show a boiler 65 which has the seams covered with enamel so as to secure a perfectly continuous enameled surface. In Buck's boiler, moreover, the cap portions, which are nearly of the diameter of the boiler, are shown as screwed to the body 70 of the boiler after the body has been enameled, and a packing is inserted in the joints made between the body and the caps. These joints are not covered with enamel, nor are the caps themselves enameled. Buck's boiler secures 75 the advantage which he sought of being readily cleaned, but does not secure the advantages which my boiler possesses, and which are hereinafter described.

My invention remedies the difficulties complained of, and I am able to produce at slight expense a very strong boiler, the interior of which, and also the exterior, if desired, is thoroughly coated with a thick surface, which adds great strength to the shell, and is not 85 nearly so liable to imperfections as other of the forms of boilers above referred to by me. Such boilers can also be made at small expense, and are very durable.

I form the outer casing or shell of my boiler 90 or similar vessel entirely of sheet metal, this being done in any ordinary manner. One of the forms is shown in the drawing, having a central cylinder and two heads lapped and riveted, the form of lapping being different 95 on the different ends. I recommend that the edges of the seam-laps should be beveled off, either by hammering, planing, or grinding, (as shown in the drawings at the top end,) before joining the parts, so as to present as 100 smooth and even a surface as possible, thus facilitating the formation of the continuous

tight and seamless coating over all parts of the vessel. I thus secure a stronger and cheaper boiler than can be made by any of the methods described in previous patents.

5 Heretofore, also, it has not been thought possible to properly coat the insides of a closed vessel—such as a boiler—with an enameling-fluid, owing to the difficulty of heating the casing uniformly by the heat of an enameling-10 furnace when parts of such casing are double at the joints formed at the laps of the seams. I secure the desired result, however, by injecting the enameling-fluid through one of the holes in the boiler, and, either by a centrifugal 15 or shaking motion, forcing the fluid over the entire interior surface of the boiler. The enameling-fluid which I use is that known as "agate," or mottled enamel for iron-ware, such as described in the patent of F. G. and

20 W. F. Niedringhaus, dated May 30, 1876, No. 177,953; reissued July 3, 1877, No. 7,779; and the manner of preparing the surface of the shell or vessel to receive such enamel and the method of applying it under ordinary circum-25 stances are now well known in the art, and, with the modification above described by me, can be successfully practiced for the purpose of my present invention.

It has been found that the agate enamel is 30 composed of such substances that it secures an extraordinary degree of attachment between the enamel and the metallic vessel to which it is applied, and it is for this reason that I prefer to use that enamel; but I do not confine 35 myself to the use of that enamel alone, because an equivalent enamel, which secures the same advantage of close connection between the metallic vessel and the enamel, thereby very greatly increasing the strength of the vessel

40 and forming a continuous enameled surface, covering the joints as well as other parts of the boiler or other vessel, and thereby securing a prevention from oxidation, and promoting, also, the facility of being cleaned, which is very 45 essential in a range-boiler, would effect my purpose. The use of this enamel is also advantageous, because range-boilers, subject as they are to alternate contraction and expansion, have been found to be very liable to

50 crack the ordinary white enamel, which has heretofore been used with such boilers to a limited extent, the "agate" enamel or its equivalent, on the contrary, being able to withstand this alternate expansion and contraction, thereby adding very materially to the 55 strength of the boiler. The enamel or glazing should be laid upon the interior surface of the metallic vessel sufficiently thickly to cover inequalities and form a strong, continuous, 60 and seamless coating, thereby rendering the vessel absolutely tight when the fluid therein contained is under pressure, and contributing

much to the durability and efficiency of the boiler. A coating of the enamel or glazing may also be applied over the whole exterior 65 of the boiler, which will accomplish to some extent the same functions as a coating on the inside, and will give to the vessel a much more ornamental appearance, and preserve it from rust, and render it much more easy to clean—an 70 important consideration where vessels of this kind are used in kitchens, where they are liable to become soiled and discolored by water and grease, and where time and labor have been necessarily employed to keep them in a 75 cleanly condition. This has been especially the case with copper boilers, which require continual scrubbing. A coating of enamel, such as described, whether inside or outside, or both, will also accomplish the following new 80 result, hitherto not practically attained by any method of production: Being tough and strong as well as possessing some material thickness, and being adherent to the surface of the metal, it not only covers over the joints 85 and renders them tight, but tends to prevent the stretching of the parts away from each other at the seams, thereby diminishing the tendency to leakage. The advantages of my boiler are, therefore, great durability, strength, 90 and tightness of the seams owing to the application of the enamel described over such seams, greater freedom from attacks of rust as compared with galvanized boilers, owing to the greater thickness of the coating in- 95 volved in the use of my material, greater cleanliness and facility for keeping clean, highly ornamental appearance, and great cheapness as compared with other boilers.

What I claim, and desire to secure by Letters Patent, is—

1. As a new article of manufacture, a range-boiler or other similar metallic vessel to be used under pressure, constructed, substantially as herein described, wholly of sheet metal, and coated on the inside with a continuous coating of enamel covering all the interior seams of the boiler, said enamel being applied after all the portions of the boiler are secured together, substantially as and for the purposes set forth. 100

2. As a new article of manufacture, a range-boiler or other similar metallic vessel to be used under pressure, constructed, substantially as herein described, wholly of sheet metal, and coated with a continuous coating of enamel 105 covering both the inside and outside of the said vessel, and extending over all the seams thereof, said enamel being applied after all the portions of the boiler are secured together, substantially as and for the purposes set forth. 115

HENRY P. FOLSOM.

Witnesses:

C. WYLLYS BETTS,  
I. R. S. BOARDMAN.